

3,503,793

### CELLULOSIC FIBROUS MATERIALS

Hans Brandeis, Limburgerhof, Pfalz, Klaus Pfleger, Ludwigshafen (Rhine), and Heinz Bille, Limburgerhof, Pfalz, Germany, assignors to Badische Anilin- & Soda-Fabrik Aktiengesellschaft, Ludwigshafen (Rhine), Germany

No Drawing. Filed Oct. 5, 1967, Ser. No. 673,015  
Claims priority, application Germany, Oct. 8, 1966,

1,594,915

Int. Cl. C09d 5/18

U.S. Cl. 117—136

3 Claims

### ABSTRACT OF THE DISCLOSURE

Fireproofing cellulosic fibrous material with compounds having the formulae



and



in which  $m$  denotes a value from 2.7 to 1.0 and  $n$  denotes a value from 1.8 to 1.0, and cellulosic material fireproofed therewith.

The present invention relates to a process for the fireproofing of cellulosic fibrous material using certain phosphorus amides and chloromethyl phosphonamides and to the cellulosic material finished in this way.

The amides, particularly the dialkylamides and the 1,2-alkylenamides of phosphoric acid and of alkylphosphonic acids and haloalkylphosphonic acids, are generally known as fireproofing agents for cellulosic fibrous material.

It is possible by means of these agents, which are in general fixed to the fibrous material by heating, to diminish the flammability of the fibrous material considerably, but usually only with impairment of other desirable properties. For example, this treatment may produce, embrittlement, a tendency to yellow of textiles finished in this way, and low resistance to washing of some of these prior art fireproofing finishes. This is especially true of the compounds giving the fireproofing effects which have hitherto been the best and most resistant to washing, namely tris-N-aziridinylphosphine oxide (phosphoric acid triethylenamide, APO) and chloromethylphosphonic bis-ethylenamide (APCI) which have the formulae:



which moreover are very toxic in the unchanged, i.e. unfixed, condition. When using other phosphoric amides and phosphonic amides (including the nontoxic compounds phosphoric-tris-methylamide and chloromethylphosphonic-bis-methylamide) good fireproofing effects are obtained but they are not resistant to washing.

The object of the present invention is to provide new fireproofing agents for cellulosic fibrous materials which give optimum and wash-resistant fireproofing effects with a minimum of deleterious secondary effects.

We have found that cellulosic fibrous materials can be given a wash-resistant fireproof finish by means of phosphoric amides of chloromethylphosphonic amides with excellent success by applying to the fibrous material a composition containing or consisting of a mixture of com-

pounds (I) and (II) defined by the following general formulae:



in which  $m$  may have any value from 2.7 to 1.0 and  $n$  may have any value from 1.8 to 1.0, these indices corresponding to the average frequency of the methylamido groups and ethylenamido groups in weighable amounts of the trivalent compounds (I) or the divalent compound (II). Thus the compounds (I) and (II) are themselves mixtures. Mixtures of (I) and (II) may also be used.

The mixtures of compounds (I) and (II), which are referred to hereinafter as compounds for simplicity, are obtainable by conventional methods, preferably by reaction of 1 mole each of phosphorus oxychloride or chloromethyl-phosphonyl dichloride with  $m$  or  $n$  moles of methylamine and  $3-m$  or  $2-n$  moles of ethylenimine in an inert organic solution at temperatures of from about  $-40^{\circ}\text{C}$ . to  $+40^{\circ}\text{C}$ . It is recommended that the solvent (for example methylene chloride, benzene, dioxane, tetrahydrofuran or ether) be placed in a reactor and the reactants be passed into the same simultaneously at the same rate in proportion to the molar composition of the product. An appropriate molar excess of methylamine, ammonia or a tertiary amine should be used to bind hydrogen chloride liberated in the reaction. Both methylammonium chloride and the hydrochlorides of tertiary amines and also ammonium chloride are insoluble in the said solvents and can be filtered off therefrom. The solution is then evaporated, advantageously at subatmospheric pressure, after which the product remains as a colorless syrupy liquid. So that it should remain stable for long periods it is advisable to dilute it, for example with water, dioxane or dimethylformamide. Compounds (I) and (II) are obtained in which the indices  $m$  and  $n$  denote only the average amounts. The mixtures of molecules formed actually have statistical distribution of the amine radicals on the phosphorus.

By "applying to the fibrous material" we mean using the flame-proofing mixture by a conventional method or any method which is known in the art.

The new agents are advantageously used in 5 to 50% aqueous solution (percentages here and hereinafter being by weight) for finishing cellulosic fibrous materials, the amount being such that the fibrous material absorbs from about 5 to 50%, preferably from 10 to 30%, of the dry weight of (I) or (II) depending on the desired intensity of the fireproofing effect. When mixtures of (I) and (II) are used, the said percentages relate to the total weight of (I) and (II). Application may be for example by dipping, spraying or padding. After the impregnated fibrous material has been dried, the agent is fixed thereon by heating for from about two to twenty minutes at about  $100^{\circ}$  to  $200^{\circ}\text{C}$ , preferably from  $150^{\circ}$  to  $170^{\circ}\text{C}$ . Following this, the fibrous material thus finished is given a conventional after-treatment for removal of unfixed agent; for example it may be washed with hot dilute aqueous alkali metal hydroxide solution or alkali metal carbonate solution.

The agents (I) and (II) which, as already stated, may be used together, are compatible with all other agents for textile finishing, particularly with a great variety of aminoplast-forming monomeric, oligomeric and polymeric compounds and may be used together with them. In other respects, the method according to this invention

may be carried out by all procedures and in all apparatus which would otherwise be used for finishing fibrous materials.

Cellulosic fibrous materials may include cotton, linen, sisal, hemp, regenerated cellulose and wood-wool in the form of filaments, threads, fibers, wadding, nonwoven fabrics or sheet materials, such as textiles and papers of all types. These materials may be mixed with others, for example wool, silk, polyester, polyamide or polyacrylonitrile, the total fireproofing effect then corresponding to that of the cellulose fraction.

The invention is further illustrated by the following examples.

#### EXAMPLE 1

A cotton cloth is impregnated with a 30% aqueous solution of a compound (I<sup>1</sup>) characterized by  $m=2$  so that the amount of finishing agent fixed to the cloth at 160° to 170° C. is about 22% of the dry weight of the cloth. Values for the fireproofing and resistance to washing of the finish (determined according to German standard specification DIN 53,906) are given in Table 1. DIN is the abbreviation for Deutsche Industrie Norm, a German industrial standard. DIN 53906 is equivalent to ASTM-D-1230. DIN 54011 is equivalent to ISO-R-105. The following abbreviations are used in the table:

Q=amount of compound fixed on the fiber

Q<sub>s</sub>=amount remaining on the fiber after washing three times with sodium carbonate solution at the boil in accordance with DIN 54,011

B=burning time in seconds

T=tear length in centimeters.

TABLE 1

|                | Not finished  | Finished with I <sup>1</sup><br>( $m=2$ ), percent |
|----------------|---------------|----------------------------------------------------|
| Q              |               | 22                                                 |
| Q <sub>s</sub> |               | 15.4                                               |
| B              | Burns through | 0                                                  |
| T              | do            | 8.9                                                |

These effects are as good as when using the much more toxic APO ( $m=0$ ).

The compound (I<sup>1</sup>) is prepared from the appropriate molar amounts of phosphorus oxychloride, methylamine, ethylenimine and ammonia (as acid-binding agent) in the course of two to three hours at -40° C. to +30° C. in methylene chloride. Elementary analysis of the pure syrupy product free from salts shows, within the limits of error, that the reactants are present in the molar ratio.

#### EXAMPLE 2

Two pieces of cotton cloth are impregnated respectively with a 23% and 30% aqueous solution of a compound (I<sup>2</sup>) characterized by  $m=1.8$  so that the amount of finishing agent fixed on the cloth at 150° to 170° C. is about 15% and about 20%, respectively, of the dry weight of the cloth. Values for fireproofing and resistance to washing of the finish, determined according to DIN 53,906, are given in Table 2 using the same abbreviations as in Table 1.

TABLE 2

|                | Not finished  | Finished with I <sup>2</sup><br>( $m=1.8$ ), percent | Finished with I <sup>2</sup><br>( $m=1.8$ ), percent |
|----------------|---------------|------------------------------------------------------|------------------------------------------------------|
| Q              |               | 15                                                   | 20                                                   |
| Q <sub>s</sub> |               | 13.5                                                 | 16                                                   |
| B              | Burns through | 0                                                    | 0                                                    |
| T              | do            | 11.0                                                 | 10.0                                                 |

These effects are as good as when using the much more toxic APO ( $m=0$ ).

The compound (I<sup>2</sup>) is prepared as described in Example 1, like the compound (I<sup>1</sup>).

#### EXAMPLE 3

A cotton cloth (two pieces) is impregnated with a 23% and a 30% aqueous solution of a compound (I<sup>3</sup>) characterized by  $m=1.5$  so that the amount of the finishing agent fixed on the fabric at 160° to 170° C. is about 15% and about 18% of the dry weight of the cloth, respectively.

Values for fireproofing and resistance to washing of the finish determined according to DIN 53,906 are given in Table 3 (using the same abbreviations as in Example 1).

TABLE 3

|                | Not finished  | Finished with I <sup>3</sup><br>( $m=1.5$ ), percent | Not finished  | Finished with I <sup>3</sup><br>( $m=1.5$ ), percent |
|----------------|---------------|------------------------------------------------------|---------------|------------------------------------------------------|
| Q              |               | 15                                                   |               | 18                                                   |
| Q <sub>s</sub> |               | 13.5                                                 |               | 14.5                                                 |
| B              | Burns through | 0                                                    | Burns through | 0                                                    |
| T              | do            | 10.1                                                 | do            | 8.4                                                  |

These effects are as good as when using the much more toxic APO ( $m=0$ ).

The compound (I<sup>3</sup>) is prepared like the compound (I<sup>1</sup>) according to Example 1.

#### EXAMPLE 4

A cotton cloth is impregnated with a 25% aqueous solution of a compound (II<sup>1</sup>) characterized by  $n=1$  so that the amount of finishing agent fixed on the cloth at 155° to 170° C. is about 18% of the dry weight of the cloth.

Values determined according to DIN 53,906 for fireproofing and resistance to washing of the finish are given in Table 4, by reference to the extent of carbonization in centimeters. The following abbreviations are used in Table 4:

T=tear length in cm without washing

T<sub>w</sub>=tear length in cm after washing with water at 60° C.

1T<sub>ss</sub>=tear length after a single wash at the boil with soap and soda

3T<sub>ss</sub>=tear length after washing three times at the boil with soap and soda.

TABLE 4

|                  | Without finishing | Finished with II <sup>1</sup><br>( $n=1$ ) |
|------------------|-------------------|--------------------------------------------|
| T                | More than 30      | 7                                          |
| T <sub>w</sub>   |                   | 8                                          |
| 1T <sub>ss</sub> |                   | 9                                          |
| 3T <sub>ss</sub> |                   | 11                                         |

These effects are as good as when using the much more toxic APCl ( $n=0$ ).

The compound (II<sup>1</sup>) is prepared like the compound (I<sup>1</sup>) as described in Example 1, substituting chloromethylphosphonyldichloride for phosphorus oxychloride.

#### EXAMPLE 5

A cotton cloth is impregnated with a 24% aqueous solution of a compound (II<sup>2</sup>) characterized by  $n=1.4$  so that the amount of finishing agent fixed on the cloth at 160° to 170° C. is about 18% of the dry weight of the cloth. (Sample A.)

Another sample of the cloth, in a further experiment, is finished in an analogous manner with the addition of 4% of hexamethoxymethylmelamine. (Sample B.)

Values (determined according to DIN 53,906) for the fireproofing and resistance to washing of the finish are given in Table 5. The Table gives the values for tear length in cm after three washes at the boil according to DIN 54,011:

TABLE 5

|          | Without any finish: | Burns Through |
|----------|---------------------|---------------|
| Sample A |                     | 11            |
| Sample B |                     | 8             |

These effects are as good as when the much more toxic APCI ( $n=$ zero) is used.

The compound (II<sup>2</sup>) is prepared like the compound (I<sup>1</sup>) as described in Example 1, substituting chloromethylphosphonyldichloride for phosphorus oxychloride.

We claim:

1. Fireproofed fibrous material consisting of or containing cellulose which has been finished with 10-30% by weight, with reference to the cellulose, of a mixture of compounds having one or both of the Formulae I and II:



in which  $m$  denotes any value from 2.7 to 1.0 and  $n$  denotes any value from 1.8 to 1.0 and these indices correspond to the average frequency of the methylamido

groups and ethylenamido groups in weighable amounts of said compounds.

2. Fireproof fibrous material as claimed in claim 1, wherein said compounds consist essentially of compounds having the Formula I.

5 3. Fireproof fibrous material as claimed in claim 1, wherein said compounds consist essentially of compounds having the Formula II.

10

15

20

#### References Cited

##### UNITED STATES PATENTS

2,891,877 6/1959 Chance et al. ----- 117—136  
3,205,034 9/1965 Chance ----- 117—136 X

##### FOREIGN PATENTS

892,131 3/1962 Great Britain.

WILLIAM D. MARTIN, Primary Examiner  
H. J. GWINNELL, Assistant Examiner

U.S. Cl. X.R.

117—143; 252—8.1

UNITED STATES PATENT OFFICE  
CERTIFICATE OF CORRECTIONPatent No. 3,503,793 Dated March 31, 1970Inventor(s) Hans Brandeis et al

It is certified that error appears in the above-identified patent and that said Letters Patent are hereby corrected as shown below:

Column 2, line 18, "(I))" should read --(II)--.

Column 5, claim 1, formula I, that portion of the formula reading "CH<sub>2</sub>" should read --  $\begin{array}{c} \text{CH}_2 \\ || \\ \text{CH}_2 \end{array}$  -- .

SIGNED AND  
SEALED

JUL 21 1970

(SEAL)

Attest:

Edward M. Fletcher, Jr.  
Attesting Officer

WILLIAM E. SCHUYLER, JR.  
Commissioner of Patents